

Feb. 27, 1962

R. D. WYLIE

3,023,098

LOW CARBON FERRITIC STAINLESS STEEL

Filed Nov. 3, 1958

2 Sheets-Sheet 1



FIG.1

INVENTOR.  
Robert D. Wylie  
BY  
J. P. Moran  
ATTORNEY

Feb. 27, 1962

R. D. WYLIE

3,023,098

LOW CARBON FERRITIC STAINLESS STEEL

Filed Nov. 3, 1958

2 Sheets-Sheet 2



FIG. 2

INVENTOR.  
Robert D. Wylie  
BY  
*J. Moran*  
ATTORNEY

# United States Patent Office

3,023,098

Patented Feb. 27, 1962

1

3,023,098

LOW CARBON FERRITIC STAINLESS STEEL  
Robert D. Wylie, Barberton, Ohio, assignor to The Bab-  
cock & Wilcox Company, New York, N.Y., a corpora-  
tion of New Jersey

Filed Nov. 3, 1958, Ser. No. 771,392

10 Claims. (Cl. 75—125)

This invention relates to ferritic alloy steels of the stainless type and, more particularly, to ferritic alloy steels of this type particularly adaptable for use in heat exchangers and related equipment where the metal may be subjected to contact with corrosive liquid or vapor either simultaneously or in alternation.

In many heat exchanger installations, certain factors, such as high temperatures and stress, for example, dictate the use of austenitic stainless steels. Such steels are used, for example, in nuclear power generating equipment. However, it has been noted that there is a tendency for austenitic stainless steels of the chromium-nickel type to be subject to stress corrosion cracking, particularly when such steels are in contact with aqueous media containing very small concentration of chloride ions, and particularly in zones where liquid or vapor are either coexisting or are alternately present. Stresses in these austenitic stainless steels, due to tube expanding, welding, and operating conditions, have been known to produce failures.

The amount of austenitic stainless steel alloys required in steam generating units has been increasing as design specifications have become more demanding. Due to the cost of these materials, investigations have been aimed toward the development of alloys having equivalent or better physical and mechanical properties but which are more economical in first cost than the austenitic stainless steels. This demand for more economic alloys has been accentuated by the stringent requirements of nuclear reactor design as well as of conventional design fossil fuel-fired steam generating units.

Heat exchangers for certain special propulsion systems require an unusual degree of integrity under operating conditions which are much more severe than those usually encountered. These heat exchangers must have welded connections between the tube and tube sheets, and these welded connections result in configurations which are susceptible to stress corrosion. Recent developments have indicated that failures in the general area of the welded connections, may be associated with stress corrosion, which may be aggravated by thermal shock. It further appears that austenitic stainless steels are particularly susceptible to this type of failure.

On the other hand, chromium stainless steels of the ferritic or martensitic type, while substantially less expensive than the austenitic stainless steels, have not found favor for high temperature, high pressure installations due to the mechanical properties of these ferritic steels and the effects of fabrication on these properties. However, it is known that these ferritic chromium stainless steels have a greater resistance to stress corrosion cracking, particularly of the type occurring when the steels are subjected with liquids and vapors including small concentrations of chloride ions.

In accordance with the present invention, a ferritic stainless steel is provided which is easy to fabricate into articles such as tubing by conventional apparatus and procedures, as compared to the difficulties and expense encountered in fabricating austenitic stainless steels, has high tensile, yield and stress-rupture strengths properties at moderately elevated temperatures, excellent elongation and ductility properties, and stress corrosion resistance properties exceeding those of austenitic stainless steels. This ferritic stainless alloy has a nominal composition of 15 Cr and 1 Ni with a carbon content not exceeding

2

0.035 and containing Mn and Si with or without purposeful additions of Mo and/or Cu.

For an understanding of the invention principles, reference is made to the following description of typical embodiments thereof as illustrated in the accompanying drawings. In the drawings:

FIGS. 1 and 2 are graphical representations of physical properties of the ferritic stainless steel alloy of the invention.

10 Ferritic stainless steel alloys of the invention have compositions within the following range of percentages by weight.

|       |                                       |
|-------|---------------------------------------|
| C     | 0.03 max. (ladle) 0.035 max. (check). |
| Cr    | 14.00 to 17.00.                       |
| Ni    | 1.00 to 1.50.                         |
| Mn    | 0.30 to 0.90.                         |
| Si    | 0.75 max.                             |
| S     | 0.03 max.                             |
| P     | 0.03 max.                             |
| 20 Cu | 0.00 to 1.10.                         |
| Mo    | 0.00 to 0.60.                         |

balance iron with the usual impurities. Where Cu is added, the percentage by weight is preferably in the range from 0.90 to 1.10 and, where Mo is added, the percentage by weight is preferably in the range from 0.40 to 0.60.

25 Within this range are ferritic stainless steel alloys having percentage by weight compositions as follows:

| Alloy No. | 1     | 2     | 3     | 4     | 5     | 6     |
|-----------|-------|-------|-------|-------|-------|-------|
| C         | 0.032 | 0.022 | 0.018 | 0.024 | 0.026 | 0.032 |
| Cr        | 16.75 | 16.50 | 15.84 | 15.72 | 15.37 | 15.14 |
| Ni        | 1.09  | 1.02  | 1.42  | 1.16  | 1.09  | 1.13  |
| Mn        | 0.71  | 0.51  | 0.74  | 0.90  | 0.67  | 0.76  |
| Si        | 0.24  | 0.25  | 0.31  | 0.44  | 0.41  | 0.24  |
| S         | 0.023 | 0.021 | 0.017 | 0.008 | 0.016 | —     |
| P         | 0.016 | 0.020 | 0.010 | 0.010 | 0.010 | —     |
| Cu        | —     | —     | 0.90  | —     | 0.10  | —     |
| Mo        | 0.51  | —     | —     | 0.49  | 0.09  | —     |

In each alloy, the balance is iron with the usual impurities.

40 A preferred ferritic stainless steel alloy embodying the invention has the following percentage composition by weight:

|      |                                       |
|------|---------------------------------------|
| C    | 0.03 max. (ladle) 0.035 max. (check). |
| Cr   | 14.00 to 16.00.                       |
| Ni   | 1.00 to 1.50.                         |
| Mn   | 0.75 max.                             |
| Si   | 0.50 max.                             |
| S    | 0.030 max.                            |
| 50 P | 0.030 max.                            |

balance iron with the usual impurities.

The ferritic stainless steel alloys embodying the invention have the following physical values when tested in the form of tubing:

|                                        | Spreads        |
|----------------------------------------|----------------|
| Tensile strength in p.s.i.             | 65,900-115,000 |
| Yield strength (0.2% offset) in p.s.i. | 47,500-102,900 |
| Percent elongation in 2"               | 20-44          |
| Hardness                               | RB 68-94       |

60 When tested in the form of forged round and plate material, using 0.505" test specimens, the alloy steels have the following physical properties:

|                                        | Spreads        |
|----------------------------------------|----------------|
| Tensile strength in p.s.i.             | 80,370-101,500 |
| Yield strength (0.2% offset) in p.s.i. | 57,930-83,000  |
| Percent elongation in 2"               | 25-31.0        |
| Percent reduction of area              | 65.6-81.1      |

70 The characteristics of the invention alloy steels when subjected to tension for short intervals at high temperatures are illustrated in FIG. 1 of the drawing. The graph

of FIG. 1 was prepared from the following table representing these different characteristics of the alloy steels:

| Test temp., ° F. | Yield strength 0.2% offset ×1,000 p.s.i. | Tensile strength ×1,000 p.s.i. | Percent elong. in 2" | Percent red. of area | Number of heats | Number of tests |
|------------------|------------------------------------------|--------------------------------|----------------------|----------------------|-----------------|-----------------|
| 400              | 47.7-66.4                                | 65.1-81.8                      | 21.2-28.5            | 67.8-75.0            | 3               | 7               |
| 500              | 43.5-57.9                                | 64.6-80.5                      | 19-28.5              | 70.7-76.6            | 2               | 8               |
| 600              | 43.8-64.0                                | 62.3-78.6                      | 18-28                | 64.9-75.1            | 3               | 8               |
| 700              | 43.4-55.1                                | 60.8-76.8                      | 19-26.5              | 65.0-74.4            | 2               | 7               |
| 800              | 58.8                                     | 69.8                           | 20.5                 | 64.6                 | 1               | 1               |

FIG. 2 graphically illustrates the stress rupture properties of a wrought bar of an alloy incorporating the invention, when subjected to normalizing at 1700° F., followed by air cooling, drawing at 1300° F., and furnace cooling. The stress rupture values of FIG. 2 are all taken at 900° F. and from the following table:

| Applied stress, p.s.i. | Rupture time, hours | Percent elongation in 2" | Percent reduction of area |
|------------------------|---------------------|--------------------------|---------------------------|
| 35,000                 | 257.2               | 40.5                     | 80.1                      |
| 32,000                 | 1,666               | 41.5                     | 74.5                      |
| 30,000                 | 5,400 to date       |                          |                           |
| 28,000                 | 3,450 removed       |                          |                           |

The following Charpy V-notch impact values are from various alloys embodying the invention which have been given certain heat treatments after forging and/or rolling operations:

(a) Forged and rolled:

| Test temp., ° F.: | Values observed, ft.-lbs. | 35 |
|-------------------|---------------------------|----|
| +10               | 103                       |    |
| -20               | 52, 68                    |    |
| -50               | 44, 70                    |    |

(b) Normalized at 1700° F., drawn at temperature from 1150° F. to 1400° F., tested at room temperature.

23 specimens—values range from 83 to 110 ft.-lbs. with an average of 92.5 ft. lbs.

(c) Normalized at 1700° F., drawn at 1300° F., stress relieved at 1350° F.:

| Test temp., ° F.: | Ft.-lbs. impact values | 45 |
|-------------------|------------------------|----|
| Room temp.        | 50, 55                 |    |
| +10               | 31, 27, 55             |    |

After 1000 hours at 885° F. as an embrittlement test the following values were observed:

| Room temp. | 38, 40, 44 | 50 |
|------------|------------|----|
| +10        | 36, 37, 38 |    |

The alloy steels of the invention have also been tested in the form of weld deposits having compositions according to the invention. The following is a tabulation of the properties of the weld deposits:

|                                                  | As welded       | After various stress relief | 60 |
|--------------------------------------------------|-----------------|-----------------------------|----|
| Tensile strength, p.s.i.                         | 101,000-115,000 | 87,000-120,000              |    |
| Yield strength (0.2% offset), p.s.i.             | 44,500-100,000  | 65,000-114,000              |    |
| Percent elongation in 2"                         | 1.1-3.0         | 16-21.5                     |    |
| Percent red. of area                             | 1.1-1.4         | 35.9-65.2                   |    |
| Weld metal impact (Charpy V-notch test) ft. lbs. | 0-6             |                             | 65 |

Insofar as corrosion resistance of the invention alloys is concerned, the corrosion rate in high purity water is less than that of carbon steel but somewhat greater than that of Type 347 austenitic stainless steels. In oxygenated water tests, the corrosion rate of the invention steels is very much better than that of carbon steels. However, when subjected to chloride containing water, the invention alloys have a stress corrosion resistance very much better than that of Type 347 and Type 304 austenitic stainless steels. Typical examples of these tests are as follows:

tenitic stainless steels. Typical examples of these tests are as follows:

(1)  $MgCl_2$  media

5 (a) Conditions:  
60 weight percent  $MgCl_2 \cdot 6H_2O$   
Boils about 220° F.  
35,000 p.s.i.

Tension type—bar specimen  
380 hours  
Results:

Type 347—severely cracked  
Invention alloys—no cracking, no pitting

15 (b) Conditions:  
42%  $MgCl_2$  by weight  
309° F. boiling point  
Horseshoe bend specimens  
75% of yield after initial bending

|                                                                                               | Treatment | Number of samples | Results                                                       |
|-----------------------------------------------------------------------------------------------|-----------|-------------------|---------------------------------------------------------------|
| Hot rolled                                                                                    |           | 7                 | 6 cracked; 1 uncracked at 500 hrs.                            |
| Annealed (after bending)                                                                      |           | 2                 | 2 uncracked at 1,025 hrs.                                     |
| Normalized and tempered (after bending)                                                       |           | 14                | 2 cracked; 4 uncracked at 500 hrs.; 8 uncracked at 1,000 hrs. |
| Normalized, tempered and stress relieved (norm. and temp. before bending, S.R. after bending) |           | 6                 | 6 uncracked at 500 hrs.                                       |

(2) Simulated boiler water tests

(a) Conditions:  
Standard Navy Boiler water  
500 p.p.m. Cl ion  
0.0 p.p.m.  $O_2$   
500° F.  
500 hours  
2 samples—both uncracked

40 (b) Conditions:  
Tilting autoclave  
50 p.p.m. Cl ion, also 500 p.p.m. NaCl  
50 p.p.m.  $PO_4$  ion  
5 p.p.m.  $SO_4$  ion  
pH 10-11 with NaOH  
Oxygen-saturated at room temperature  
485° F.

600 p.s.i.g.  
24 hours  
U bend tube samples and straight retractively expanded tubes

Samples suspended in vapor phase  
Minimum of 50 wettings of 25-30 seconds duration in 24 hour run.  
Results:

Type 347—  
13 U bends—13 cracked  
12 expanded tubes—12 cracked  
Invention alloys—  
32 U bends—None cracked  
10 expanded tubes—None cracked  
Remarks—Type 347 exhibits typical stress corrosion cracks.  
Invention alloy exhibits some pitting tendencies.  
However, certain passivation treatments resulted in excellent pitting resistance.

Metallographic examination of the invention alloy in the form of tubing and extruded bar stock, and in the process annealed condition, reveals a fine grained microstructure of tempered martensite and ferrite. The microstructure contains approximately 50 percent martensite, which enhances the mechanical properties of the alloy, such as tensile strength and hardness properties, and increases its impact strength, particularly as compared to

alloys having a microstructure which is preponderantly ferrite.

While specific embodiments of the invention have been shown and described in detail to illustrate the application of the invention principles, it will be understood that the invention may be embodied otherwise without departing from such principles.

What is claimed is:

1. An alloy steel resistant to stress corrosion cracking when subjected to corrosive atmospheres and having good impact strength at low temperatures, excellent mechanical properties at moderately elevated temperatures, and characterized by a fine-grained microstructure of tempered martensite and ferrite, the martensite constituting approximately 50 percent of the microstructure; said alloy steel having the following percentage composition by weight:

|    |                |
|----|----------------|
| Cr | 14.00 to 16.75 |
| Ni | 1.02 to 1.50   |
| C  | 0.018 to 0.035 |
| Mn | 0.51 to 0.90   |
| Si | 0.24 to 0.50   |
| S  | 0.030 max.     |
| P  | 0.030 max.     |
| Cu | Up to 0.90     |
| Mo | Up to 0.51     |

balance iron with the usual impurities.

2. An alloy steel resistant to stress corrosion cracking when subject to corrosive atmospheres and having good impact strength at low temperatures, excellent mechanical properties at moderately elevated temperatures, and characterized by a fine-grained microstructure of tempered martensite and ferrite, the martensite constituting approximately 50 percent of the microstructure; said alloy steel having the following percentage composition by weight:

|    |       |    |       |
|----|-------|----|-------|
| Cr | 16.75 | Si | 0.24  |
| Ni | 1.09  | S  | 0.023 |
| C  | 0.032 | P  | 0.016 |
| Mn | 0.71  | Mo | 0.51  |

balance iron with the usual impurities.

3. An alloy steel resistant to stress corrosion cracking when subjected to corrosive atmospheres and having good impact strength at low temperatures, excellent mechanical properties at moderately elevated temperatures, and characterized by a fine-grained microstructure of tempered martensite and ferrite, the martensite constituting approximately 50 percent of the microstructure; said alloy steel having the following percentage composition by weight:

|    |       |    |       |
|----|-------|----|-------|
| Cr | 16.50 | Si | 0.25  |
| Ni | 1.02  | S  | 0.021 |
| C  | 0.022 | P  | 0.022 |
| Mn | 0.51  |    |       |

balance iron with the usual impurities.

4. An alloy steel resistant to stress corrosion cracking when subjected to corrosive atmospheres and having good impact strength at low temperatures, excellent mechanical properties at moderately elevated temperatures, and characterized by a fine-grained microstructure of tempered martensite and ferrite, the martensite constituting approximately 50 percent of the microstructure; said alloy steel having the following percentage composition by weight:

|    |       |    |       |
|----|-------|----|-------|
| Cr | 15.84 | Si | 0.31  |
| Ni | 1.42  | S  | 0.017 |
| C  | 0.018 | P  | 0.010 |
| Mn | 0.74  | Cu | 0.90  |

balance iron with the usual impurities.

5. An alloy steel resistant to stress corrosion cracking when subjected to corrosive atmospheres and having good impact strength at low temperatures, excellent mechanical properties at moderately elevated temperatures, and char-

acterized by a fine-grained microstructure of tempered martensite and ferrite, the martensite constituting approximately 50 percent of the microstructure; said alloy steel having the following percentage composition by weight:

|    |       |    |       |
|----|-------|----|-------|
| Cr | 15.72 | Si | 0.44  |
| Ni | 1.16  | S  | 0.008 |
| C  | 0.024 | P  | 0.010 |
| Mn | 0.90  | Mo | 0.49  |

balance iron with the usual impurities.

6. An alloy steel resistant to stress corrosion cracking when subjected to corrosive atmospheres and having good impact strength at low temperatures, excellent mechanical properties at moderately elevated temperatures, and characterized by a fine-grained microstructure of tempered martensite and ferrite, the martensite constituting approximately 50 percent of the microstructure; said alloy steel having the following percentage composition by weight:

|    |       |    |       |
|----|-------|----|-------|
| Cr | 15.37 | S  | 0.016 |
| Ni | 1.09  | P  | 0.010 |
| C  | 0.026 | Cu | 0.10  |
| Mn | 0.67  | Mo | 0.09  |
| Si | 0.41  |    |       |

balance iron with the usual impurities.

7. An alloy steel resistant to stress corrosion cracking when subjected to corrosive atmospheres and having good impact strength at low temperatures, excellent mechanical properties at moderately elevated temperatures, and characterized by a fine-grained microstructure of tempered martensite and ferrite, the martensite constituting approximately 50 percent of the microstructure; said alloy having the following percentage composition by weight:

|    |       |    |      |
|----|-------|----|------|
| Cr | 15.14 | Mn | 0.76 |
| Ni | 1.13  | Si | 0.24 |
| C  | 0.032 |    |      |

balance iron with the usual impurities.

8. An alloy steel resistant to stress corrosion cracking when subjected to corrosive atmospheres and having good impact strength at low temperatures, excellent mechanical properties at moderately elevated temperatures, and characterized by a microstructure of martensite and ferrite; said alloy steel having the following percentage composition by weight:

|    |              |
|----|--------------|
| Cr | 14.0 to 16.0 |
| Ni | 1.0 to 1.5   |
| C  | 0.035 max.   |
| Mn | 0.75 max.    |
| Si | 0.50 max.    |
| S  | 0.030 max.   |
| P  | 0.030 max.   |

balance iron with the usual impurities.

9. An alloy steel resistant to stress corrosion cracking when subjected to corrosive atmospheres and having good impact strength at low temperatures, excellent mechanical properties at moderately elevated temperatures, and characterized by a fine-grained microstructure of tempered martensite and ferrite, the martensite constituting approximately 50 percent of the microstructure; said alloy steel having the following percentage composition by weight:

|    |              |
|----|--------------|
| Cr | 14.0 to 16.0 |
| Ni | 1.0 to 1.5   |
| C  | 0.035 max.   |
| Mn | 0.75 max.    |
| Si | 0.50 max.    |
| S  | 0.030 max.   |
| P  | 0.030 max.   |

balance iron with the usual impurities.

10. An alloy steel resistant to stress corrosion cracking when subjected to corrosive atmospheres and having good impact strength at low temperatures, good weldability, excellent mechanical properties at moderately elevated

temperatures, and characterized by a microstructure of martensite and ferrite; said alloy steel having the following percentage composition by weight:

|    |                |    |
|----|----------------|----|
| Cr | 14.00 to 17.00 | 5  |
| Ni | 1.00 to 1.50   |    |
| C  | 0.035 max.     |    |
| Mn | 0.30 to 0.90   |    |
| Si | 0.75 max.      |    |
| S  | 0.030 max.     | 10 |
| P  | 0.030 max.     |    |
| Cu | up to 1.10     |    |
| Mo | up to 0.60     |    |

and balance iron with the usual impurities.

References Cited in the file of this patent

UNITED STATES PATENTS

|           |           |               |
|-----------|-----------|---------------|
| 1,441,479 | Bennett   | Jan. 9, 1923  |
| 1,630,448 | Oertel    | May 31, 1927  |
| 1,775,615 | Succop    | Sept. 9, 1930 |
| 2,310,341 | Arness    | Feb. 9, 1943  |
| 2,362,277 | Jones     | Nov. 7, 1944  |
| 2,851,384 | Waxweiler | Sept. 9, 1958 |

OTHER REFERENCES

Metal Handbook, 1954 Supplement, pages 34-39; published by The American Society of Metals, Cleveland, Ohio (first published as the July 15, 1954, issue of Metals Progress).